# EUROPEAN PATENT SPECIFICATION

(11) **EP 4 105 381 B1**
(45) Date of publication and mention of the grant of the patent: **31.05.2023**
(21) Application number: 21180362.2
(22) Date of filing: 18.06.2021
(51) Int. Cl.: D21H 11/08, D21H 11/10, D21H 11/14, D21H 27/30

(54) **PRODUCT OF PAPERBOARD HAVING IMPROVED PRINTING PROPERTIES**
PRODUKT AUS PAPPE MIT VERBESSERTEN DRUCKEIGENSCHAFTEN
PRODUIT DE CARTON PRÉSENTANT DE MEILLEURES PROPRIÉTÉS D'IMPRESSION

(43) Date of publication of application: 21.12.2022
(73) Proprietor: Billerud Aktiebolag (publ), 169 27 Solna (SE)
(72) Inventor: LINDSTEDT, Thomas, 653 45 KARLSTAD (SE); ERICSSON, Stefan, 731 92 KÖPING (SE)
(74) Representative: Kransell & Wennborg KB

(56) References cited:
- EP-A1- 1 936 032
- EP-A1- 3 805 453
- WO-A1-2009/153225
- WO-A1-2016/140609
- WO-A1-2017/006216
- WO-A1-2019/180303
- WO-A1-2021/059219
- US-A1- 2004 099 388

## Description

### TECHNICAL FIELD

The present disclosure relates to the field of paperboard production.

### BACKGROUND

Paperboard often has several layers, including a top layer intended to be printed, a bottom/reverse layer and at least one middle layer. The top layer is often provided with a pigment coating to improve printing properties. To obtain high bending stiffness at a relatively low consumption of cellulose fibres, the middle layer(s) typically have relatively high bulk (i.e., low density). To achieve high bulk, CTMP is often included in the pulp mixture used to form the middle layer. CTMP is traditionally formed from softwood (e.g., spruce). The type of pulp used for forming the top and the bottom layer has been mainly kraft pulp.

EP1936032A1 relates to a method of producing a laminate paper product comprising at least two layers, said method comprising
(i) providing an aqueous suspension comprising cellulosic fibers
(ii) adding to the suspension microfibrillar polysaccharide in an amount to yield from about 0.05 to about 50 wt% based on the weight of the cellulosic fibers
(iii) dewatering the obtained suspension and forming a first layer having a density from about 150 to about 500 kg/m3 of said laminate paper product.

WO 2016/140609 relates a pulp mixture comprising a first pulp and a second pulp, the first pulp consisting of a chemical softwood pulp which has been subjected to high consistency refining followed by low consistency refining, the second pulp consisting of a bulk increasing pulp selected from the group consisting of a chemi-thermomechanical pulp (CTMP), a thermomechanical pulp (TMP) and a chemical softwood pulp which has been subjected to low consistency refining without preceding high consistency refining, and wherein: in the case the second pulp is a CTMP or a TMP, the first pulp is present in an amount of 20-90 %, such as 25-90 %, such as 50-90 % by dry weight of the total dry weight of the first pulp and the second pulp; in the case the second pulp is a chemical softwood pulp which has been subjected to a low consistency refining without preceding high consistency refining, the first pulp is present in an amount of 5-90 % by dry weight of the total dry weight of the first pulp and the second pulp.

WO 2009/153225 relates to a process of producing a cellulosic product comprising (i) providing an aqueous suspension of cellulosic fibers, (ii) adding microfibrillar polysaccharide, (iii) adding thermoplastic microspheres, (iv) dewatering the suspension and forming a cellulosic product. It also relates to a process of producing a single layer cellulosic product comprising (i) providing an aqueous suspension of cellulosic fibers, (ii) adding microfibrillar polysaccharide derived from softwood and/or hardwood and optionally adding thermoplastic microspheres to the suspension, (iii) dewatering the suspension and forming a cellulosic product.

### SUMMARY

High headbox consistency is generally associated with poor printing properties. This is not only the case for the headbox consistency used for forming the top/printing layer, but also for the headbox consistency used for forming the middle layer arranged below the top/printing layer. Still, it is advisable to have a relatively high headbox consistency in some methods of making paperboard, e.g., when the headbox have a certain design (i.e., the energy-efficient "low turbulence" design used by headbox suppliers Escher Wyss and now Voith), when middle layers of higher grammages are formed and/or to facilitate higher machine speeds.

The present inventors have realized that the printing properties should not be improved by lowering the headbox consistency, but by modifying the composition of the middle layer furnish. However, the modified furnish should still produce a middle layer that meet other paperboard requirements.

The present invention is defined in the current claim 1. Accordingly, there is provided a method of forming a multi-layered paperboard comprising a bottom layer, a top layer and a middle layer arranged between the top layer and the bottom layer, wherein the middle layer is formed from a middle layer furnish comprising at least 30% by dry weight of a HT-CTMP from a mixture of hardwood and softwood, which middle layer furnish is fed to a wire from a middle layer head box in which the consistency is above 0.30%, such as above 0.40%, such as at least 0.43%.

### DETAILED DESCRIPTION

The present disclosure provides a method of forming a multi-layered paperboard comprising a bottom layer, a top layer and a middle layer. As understood by the skilled person, the middle layer is arranged between the top layer and the bottom layer. Normally, the middle layer has a lower density than the top layer and the bottom layer. The top layer is typically intended for printing and may thus be covered by a pigment coating. The pigment coating may have one or more layers, such as one, two or three layers. In one embodiment, also the bottom layer is covered by a pigment coating. The total coat weight (dry) of the pigment coating provided on the top layer may be 10-40 g/m². The coat weight (dry) of the pigment coating provided on the bottom layer may be 4-15 g/m², such as 5-10 g/m². Application of coating compositions is further discussed below.

The method is preferably carried out in a full-scale paperboard machine comprising a forming section, a pressing section and a drying section. The full-scale paperboard machine may further comprise a coating section arranged downstream the drying section. In one embodiment, the full-scale paperboard machine comprises at least on calender arranged downstream the drying section or in a downstream region of the drying section. When the coating section is included, the calender is typically arranged upstream thereof. A full-scale paperboard machine typically produces at least 50,000 tonnes of paperboard per year.

The middle layer is formed from a middle layer furnish comprising at least 30% by dry weight of a HT-CTMP characterized by that it is formed from a mixture of hardwood and softwood. In one embodiment, the middle layer furnish comprises at least 35% by dry weight of the HT-CTMP, such as at least 40% by dry weight of the HT-CTMP. A typical upper limit may be 60% by dry weight.

The hardwood may be aspen, birch or eucalyptus.

The term HT-CTMP (high-temperature chemithermomechanical pulp) refers to CTMP that has, during the production thereof, been heated to a temperature of at least 140 °C, preferably of at least 150 °C, more preferably of at least 160 °C, prior to the refining step.

The Canadian Standard Freeness measured according to ISO 5267-2:2001 of the HT-CTMP may be 500-650 ml, such as 530-630 ml. The HT-CTMP may be bleached.

The middle layer furnish may further comprise broke pulp, such as at least 30% (by dry weight) of a broke pulp, such as at least 40% (by dry weight) of a broke pulp.

The Schopper-Riegler number measured according to ISO 5267-1:1999 of the broke pulp may be 26-34, such as 28-32.

In one embodiment, the middle layer furnish further comprises chemical pulp, such as 5-25% (by dry weight) of a kraft pulp. The kraft pulp may be softwood kraft pulp.

To form the middle layer, the middle layer furnish is fed to a wire from a middle layer head box. In the middle layer head box, the consistency of the middle layer furnish is above 0.30%, such as above 0.40%, such as at least 0.43%. A typical upper limit for the consistency in the middle layer head box is 0.80%, such as 0.70%.

In one embodiment, the mixture comprises 20-80% softwood and 20-80% hardwood. Preferably, the hardwood is included in a higher proportion than the softwood.

In one embodiment, the grammage of the middle layer is at least 130 g/m², such as at least 140 g/m², such as at least 145 g/m². An upper limit may be 210 g/m². The papermaker knows the grammage of each layer that he/she is producing.

The grammage of the complete multi-layered paperboard (including any pigment coating(s)) may be at least 250 g/m², such as at least 260 g/m², such as at least 270 g/m². An upper limit may be 400 g/m².

The density (ISO 534:2011) of the complete multi-layered paperboard (including any pigment coating(s)) may be below 800 kg/m3, such as below 750 kg/m³, such as below 725 kg/m³. A lower limit may be 650 kg/m³.

The density (ISO 534:2011) of the middle layer may be below 625 kg/m³, such as below 600 kg/m³.

To separate the middle layer from the multi-layered paperboard and thus facilitate the density measurement, a FORTUNA Bandknife-Splitting Machine (Type AB 320 E/P) can be used. Such a machine that has been customized for paperboard splitting is commercially available and is used by several major companies in the paperboard field.

Alternatively, a surface grinding technique can be used to remove all layers but the middle layer in question. Such a surface grinding is one of the services that are commercially available at RISE Bioeconomy (formerly Innventia) in Stockholm, Sweden.

In one embodiment, the top layer is formed from a top layer furnish comprising at least 50% by dry weigh of kraft pulp, such as at least 80% by dry weigh of kraft pulp. The kraft pulp of the top layer may be bleached.

Further, the top layer furnish may comprise a mixture of hardwood pulp and softwood pulp.

In one embodiment, hardwood kraft pulp constitutes at least 80% by dry weight of the top layer furnish. In another embodiment, hardwood kraft pulp and softwood kraft pulp together constitute at least 80% by dry weight of the top layer furnish

In one embodiment, the bottom layer is formed from a bottom layer furnish comprising at least 50% by dry weigh of kraft pulp, such as at least 70% by dry weigh of kraft pulp. The kraft pulp of the bottom layer is typically softwood kraft pulp or a mixture of hardwood kraft pulp and softwood kraft pulp.

In one embodiment, the multi-layered paperboard comprises more than one middle layer arranged between the top layer and the bottom layer.

The method may comprise a step of online coating the multi-layered paperboard with at least one pigment coating composition. The coating step may comprise several sub-steps. As an example, at least two pigment coating layers may be added to the top layer in at least two sub-steps. Another sub-step may be coating of the bottom layer. Equipment suited for on-line coating of paperboard is known to the skilled person.

### EXAMPLES

### Inventive trial

An embodiment of the method of the present disclosure was carried out in full scale in a paperboard machine.

To prepare a top layer furnish, bleached hardwood kraft pulp was subjected to LC refining (75 kWh/tonne) resulting in a SR number of 30. Bleached softwood kraft pulp was also subjected to LC refining (150 kWh/tonne) resulting in a SR number of 30. After refining, the pulps were mixed in a 75/25 dry weight ratio (hardwood/softwood). Before the top layer headbox, rosin size (0.9 kg/tonne), alum (2.3 kg/tonne), strength agent (cationic starch, 2.5 kg/tonne), retention starch (3 kg/tonne), retention polymer (75 g/tonne), silica (300 g/tonne) and clay (75 kg/tonne) were added. In the top layer headbox, the consistency was 0.19% and the pH was 6.8.

To prepare a bottom layer furnish, bleached softwood kraft pulp was subjected to LC refining (70 kWh/tonne) resulting in a SR number of 20. Before the bottom layer headbox, rosin size (1.0 kg/tonne), alum (2.3 kg/tonne), strength agent (cationic starch, 2.5 kg/tonne), retention starch (3 kg/tonne), retention polymer (100 g/tonne), silica (300 g/tonne) and clay (20 kg/tonne) were added. In the bottom layer headbox, the consistency was 0.15% and the pH was 6.8.

To prepare a middle layer furnish, bleached softwood kraft pulp was subjected to LC refining (90 kWh/tonne) resulting in a SR number of 20. Further, bleached HT-CTMP formed from a mixture of hardwood and softwood was subjected to LC refining (20 kWh/tonne) resulting in a CSF of 580 ml and broke pulp was refined to the extent it obtained a SR number of 30. After refining, the pulps were mixed in a 15/40/45 dry weight ratio (softwood kraft pulp/CTMP/broke pulp). Before the middle layer headbox, rosin size (2.5 kg/tonne), alum (3.8 kg/tonne), retention starch (3 kg/tonne), retention polymer (100 g/tonne) and silica (350 g/tonne) were added. In the middle layer headbox, the consistency was 0.43% and the pH was 6.8. The wire used for forming the middle layer included a breast roll shaker.

In the wire section, 0.5 g/m² starch was sprayed to each of the top layer web and the bottom layer web for ply-bond strength. At the end of the wire section, the three individual webs were couched together to form a three-layered web. The wire speed was 583 m/min. In the press section arranged downstream the wire section, the three-layered web was pressed in three nips; a first shoe press nip (490 kN/m) followed by a second shoe press nip (750 kN/m) followed by a hard nip (50 kN/m).

Downstream the press section, the three-layered web was dried in a drying section and then calendered in a hard nip calender at a line load of 30 kN/m. After the calendering, the web was coated in a coating section having four stations. In the first station, which was a metering size press (MSP), 5 g/m² (dry) of a pigment coating composition was coated onto the top surface. In the second station, which was a blade coater, another 9 g/m² of a pigment coating composition was coated onto the top surface. In the third station, which was a metering size press (MSP), 7 g/m² of a pigment coating composition was coated onto the bottom surface. carried out in a drying section. In the fourth station, which was a blade coater, another 9 g/m² of a pigment coating composition was coated onto the top surface. Hence a total of 23 g/m² was coated onto the top surface and a total of 7 g/m² was coated onto the bottom surface.

The properties of the resulting paperboard are presented in table 1 below.

### Reference trial

The reference trial was carried out in the same way as the inventive trial presented above, but with the following exceptions:
a "normal" bleached softwood CTMP that was LC-refined to a CSF of 650 ml was used instead of the bleached HT-CTMP formed from the hardwood/softwood mixture; and
the line load in the hard nip calender was 60 kN/m instead of 30 kN/m.

The properties of the resulting paperboard are presented in table 1 below.

**Table 1**

| Property | Inventive trial | Reference trial |
|---|---|---|
| Paperboard grammage (g/m²) | 294 | 305 |
| Top layer grammage (g/m²) | 67 | 67 |
| Middle layer grammage (g/m²) | 146 | 157 |
| Bottom layer grammage (g/m²) | 51 | 51 |
| Paperboard thickness (µm) | 409 | 404 |
| Paperboard density (kg/m³) | 720 | 756 |
| Bendtsen Roughness* (ml/min) | 33.7 | 62.8 |
| PPS roughness* (µm) | 1.20 | 1.37 |
| Scott Bond (J/m²) | 168 | 232 |
| Z strength (kPa) | 357 | 375 |
| Bending stiffness (mNm) | 297 | 289 |
| Bending stiffness index (Nm⁷kg³) | 11.6 | 10.1 |
| SCT (N/m) | 8.72 | 9.36 |
| SCT index (Nm/g) | 29.7 | 30.7 |

| | | |
|---|---|---|
| * Measured on the top side | | |

As shown by table 1, the inventive trial resulted in a paperboard of at least comparable and in some cases improved properties when compared to those of the paperboard produced in the reference trial.

In addition, the inventors' impression of the outcome of the inventive trial was that it resulted in the greatest improvement of printing properties they had ever seen in a full-scale machine trial.

The inventors' impression is surprising in view of that the line load in the hard nip calender was reduced in the inventive trial compared to the reference trial and that reduced line load is normally associated with impaired printing properties.

The reduced density shown in table 1 can at least partly be explained by the reduced line load.

Notably, the taste and odour problems sometimes associated with the use of hardwood CTMP were not encountered in the inventive trial.

### Visual scoring of print quality

A panel of 12 people was recruited to visually analyse and score the print quality of seven different samples in a blinded study. Paperboard produced according to the Reference trial described above was used for samples 2 and 3. Sample 2 was obtained from a centre reel. Sample 3 was obtained from an edge reel. Paperboard produced according to the Inventive trial described above was used for samples 4 and 5. A paperboard produced according to the Inventive trial described above, but with a line load of 40 kN/m in the hard nip calender, was used for samples 6 and 7. Samples 4 and 6 were obtained from centre reels and samples 5 and 7 were obtained from edge reels. Sample 1 was obtained from paperboard produced on another paper machine using "traditional" softwood CTMP.

For each sample, two prints were made. The first print was a photograph of a woman. The second print was a photograph of a flower (a dandelion).

For each print, each panellist made pairwise visual comparisons of all samples without any knowledge of the identity of the paperboard (blinded study). For each pair, two points were awarded. If one printed sample was considered to have a better print quality than the other, it was given two points, while the other printed sample was given zero points. If the print qualities were considered to be equal, the samples were given one point each.

For each panellist, the points given to each print of each sample were then summarized (each print of each sample underwent six pairwise comparisons and could thus get from zero (0) to twelve (12) points). The results are presented in tables 2 and 3 below.

**Table 2. The first print.**

| Sample | Ref. 1 | Ref. 2 | Ref. 3 | Inventive 4 | Inventive 5 | Inventive 6 | Inventive 7 |
|---|---|---|---|---|---|---|---|
| Panellist 1 | 0 | 2 | 4 | 12 | 10 | 8 | 6 |
| Panellist 2 | 1 | 1 | 9 | 5 | 10 | 8 | 8 |
| Panellist 3 | 0 | 6 | 6 | 6 | 10 | 6 | 8 |
| Panellist 4 | 0 | 5 | 5 | 8 | 11 | 5 | 8 |
| Panellist 5 | 1 | 2 | 5 | 7 | 8 | 9 | 10 |
| Panellist 6 | 0 | 2 | 4 | 10 | 10 | 10 | 8 |
| Panellist 7 | 0 | 2 | 4 | 10 | 8 | 12 | 6 |
| Panellist 8 | 0 | 5 | 7 | 9 | 6 | 8 | 7 |
| Panellist 9 | 0 | 2 | 4 | 6 | 10 | 10 | 10 |
| Panellist 10 | 2 | 5 | 3 | 8 | 10 | 7 | 7 |
| Panellist 11 | 2 | 2 | 2 | 12 | 8 | 10 | 6 |
| Panellist 12 | 1 | 1 | 5 | 7 | 12 | 8 | 8 |
| Average score | 0.6 | 2.9 | 4.8 | 8.3 | 9.4 | 8.4 | 7.7 |

**Table 3. The second print.**

| Sample | Ref. 1 | Ref. 2 | Ref. 3 | Inventive 4 | Inventive 5 | Inventive 6 | Inventive 7 |
|---|---|---|---|---|---|---|---|
| Panellist 1 | 3 | 1 | 2 | 9 | 8 | 10 | 9 |
| Panellist 2 | 1 | 1 | 6 | 8 | 10 | 7 | 9 |
| Panellist 3 | 6 | 0 | 2 | 10 | 10 | 4 | 10 |
| Panellist 4 | 3 | 0 | 3 | 7 | 8 | 9 | 12 |
| Panellist 5 | 2 | 2 | 2 | 7 | 8 | 12 | 9 |
| Panellist 6 | 2 | 3 | 1 | 10 | 7 | 8 | 11 |
| Panellist 7 | 0 | 3 | 3 | 12 | 8 | 7 | 9 |
| Panellist 8 | 3 | 6 | 6 | 7 | 6 | 7 | 7 |
| Panellist 9 | 0 | 4 | 2 | 9 | 9 | 9 | 9 |
| Panellist 10 | 2 | 3 | 2 | 8 | 9 | 9 | 9 |
| Panellist 11 | 4 | 9 | 5 | 12 | 2 | 7 | 3 |
| Panellist 12 | 6 | 4 | 6 | 6 | 4 | 8 | 8 |
| Average score | 2.7 | 3.0 | 3.3 | 8.8 | 7.4 | 8.1 | 8.8 |

Tables 2 and 3 show that the inventive board production undoubtedly resulted in much better print quality than the references. Tables 2 and 3 thus confirm the inventors' impression discussed above.

## Claims

1. A method of forming a multi-layered paperboard comprising a bottom layer, a top layer and a middle layer arranged between the top layer and the bottom layer, wherein the middle layer is formed from a middle layer furnish comprising at least 30% by dry weight of a high-temperature chemithermomechanical pulp (HT-CTMP) from a mixture of hardwood and softwood, which middle layer furnish is fed to a wire from a middle layer head box in which the consistency is above 0.30%, such as above 0.40%, such as at least 0.43%, wherein the term HT-CTMP refers to CTMP that has, during the production thereof, been heated to a temperature of at least 140 °C, preferably of at least 150 °C, more preferably of at least 160 °C, prior to the refining step.

2. The method of claim 1, wherein the middle layer furnish comprises at least 35% by dry weight of the HT-CTMP, such as at least 40% by dry weight of the HT-CTMP.

3. The method of claim 1 or 2, wherein the middle layer furnish comprises at least 30% of a broke pulp, such as at least 40% of a broke pulp.

4. The method of any one of the preceding claims, wherein the middle layer furnish comprises 5-25% of a kraft pulp, such as a softwood kraft pulp.

5. The method of any one of the preceding claims, wherein the mixture comprises 20-80% softwood and 20-80% hardwood.

6. The method of any one of the preceding claims, wherein the grammage of the middle layer is at least 130 g/m², such as at least 140 g/m², such as at least 145 g/m²,

7. The method of any one of the preceding claims, wherein the grammage of the multi-layered paperboard is at least 250 g/m², such as at least 260 g/m², such as at least 270 g/m².

8. The method of any one of the preceding claims, wherein the density of the multi-layered paperboard is below 800 kg/m3, such as below 750 kg/m3, such as below 725 kg/m3

9. The method of any one of the preceding claims, wherein the top layer is formed from a top layer furnish comprising at least 50% by dry weigh of kraft pulp, such as at least 80% by dry weigh of kraft pulp.

10. The method of claim 9, wherein the top layer furnish comprises a mixture of hardwood pulp and softwood pulp.

11. The method of any one of the preceding claims, wherein the bottom layer is formed from a bottom layer furnish comprising at least 50% by dry weigh of kraft pulp, such as at least 70% by dry weigh of kraft pulp.

## Patentansprüche

1. Verfahren zum Bilden von mehrschichtiger Pappe, die eine untere Schicht, eine obere Schicht und eine zwischen der oberen Schicht und der unteren Schicht angeordnete mittlere Schicht aufweist, wobei die mittlere Schicht aus einem Mittelschicht-Faserstoff gebildet wird, der mindestens 30 Gew.-% Trockengewicht eines chemothermomechanischen Hochtemperatur-Zellstoffs (HT-CTMP) aus einer Mischung aus Hartholz und Weichholz aufweist, dessen Mittelschicht-Faserstoff einem Sieb aus einem Mittelschicht-Stoffauflaufkasten zugeführt wird, in dem die Konsistenz über 0,30 %, beispielsweise über 0,40 %, beispielsweise mindestens 0,43 %, liegt, wobei sich der Begriff HT-CTMP auf einen CTMP bezieht, das während seiner Herstellung auf eine Temperatur von mindestens 140 °C, vorzugsweise mindestens 150 °C, mehr bevorzugt mindestens 160 °C, vor dem Raffinationsschritt erhitzt wurde.

2. Verfahren nach Anspruch 1, wobei der Mittelschicht-Faserstoff mindestens 35 Gew.-% Trockengewicht des HT-CTMP, wie beispielsweise mindestens 40 Gew.-% Trockengewicht des HT-CTMP, aufweist.

3. Verfahren nach Anspruch 1 oder 2, wobei der Mittelschicht-Faserstoff mindestens 30 % Ausschusszellstoff, beispielsweise mindestens 40 % Ausschusszellstoff, aufweist.

4. Verfahren nach einem der vorhergehenden Ansprüche, wobei der Mittelschicht-Faserstoff 5-25 % Kraftzellstoff, beispielsweise Weichholz-Kraftzellstoff, aufweist.

5. Verfahren nach einem der vorhergehenden Ansprüche, wobei die Mischung 20-80 % Weichholz und 20-80 % Hartholz aufweist.

6. Verfahren nach einem der vorhergehenden Ansprüche, wobei das Flächengewicht der Mittelschicht mindestens 130 g/m², beispielsweise mindestens 140 g/m², beispielsweise mindestens 145 g/m², beträgt.

7. Verfahren nach einem der vorhergehenden Ansprüche, wobei das Flächengewicht der mehrschichtigen Pappe mindestens 250 g/m², beispielsweise mindestens 260 g/m², beispielsweise mindestens 270 g/m², beträgt.

8. Verfahren nach einem der vorhergehenden Ansprüche, wobei die Dichte der mehrschichtigen Pappe unter 800 kg/m3, beispielsweise unter 750 kg/m3, beispielsweise unter 725 kg/m3, liegt.

9. Verfahren nach einem der vorhergehenden Ansprüche, wobei die obere Schicht aus einem Oberschichtstoff gebildet wird, der mindestens 50 Gew-% Trockengewicht Kraftzellstoff, beispielsweise mindestens 80 Gew-% Trockengewicht Kraftzellstoff, aufweist.

10. Verfahren nach Anspruch 9, wobei der Faserstoff der oberen Schicht eine Mischung aus Hartholzzellstoff und Weichholzzellstoff aufweist.

11. Verfahren nach einem der vorhergehenden Ansprüche, wobei die untere Schicht aus einem Unterschichtstoff gebildet wird, der mindestens 50 Gew-% Trockengewicht Kraftzellstoff, beispielsweise mindestens 70 Gew-% Trockengewicht Kraftzellstoff, aufweist.

## Revendications

1. Procédé de formation d'un carton multicouche comprenant une couche inférieure, une couche supérieure et une couche intermédiaire disposée entre la couche supérieure et la couche inférieure, dans lequel la couche intermédiaire est formée à partir d'une pâte intermédiaire comprenant au moins 30 % en poids sec d'une pâte chimicomécanique à haute température (HT-CTMP) provenant d'un mélange de bois feuillus et de bois résineux, cette pâte de couche intermédiaire est introduite dans un fil à partir d'une caisse de tête de couche intermédiaire dans laquelle la consistance est supérieure à 0,30 %, telle que supérieure à 0,40 %, telle que supérieure à 0,43 %, dans lequel le terme HT-CTMP fait référence à une CTMP qui, au cours de sa production, a été chauffée à une température d'au moins 140 °C, de préférence d'au moins 150 °C, plus préférentiellement d'au moins 160 °C, avant l'étape de raffinage.

2. Procédé selon la revendication 1, dans lequel la couche intermédiaire comprend au moins 35 % en poids sec de la HT-CTMP, par exemple au moins 40 % en poids sec de la HT-CTMP.

3. Procédé selon la revendication 1 ou la revendication 2, dans lequel la couche intermédiaire comprend au moins 30 % de pâte brisée, telle qu'au moins 40 % de pâte brisée.

4. Procédé selon l'une quelconque des revendications précédentes, dans lequel la couche intermédiaire comprend de 5 à 25 % de pâte kraft, telle que de la pâte kraft de bois tendre.

5. Procédé selon l'une quelconque des revendications précédentes, dans lequel le mélange comprend de 20 à 80 % de bois dur et de 20 à 80 % de bois tendre.

6. Procédé selon l'une quelconque des revendications précédentes, dans lequel le grammage de la couche intermédiaire est d'au moins 130 g/m², tel qu'au moins 140 g/m², tel qu'au moins 145 g/m².

7. Procédé selon l'une quelconque des revendications précédentes, dans lequel le grammage du carton multicouche est d'au moins 250 g/m², tel qu'au moins 260 g/m², tel qu'au moins 270 g/m².

8. Procédé selon l'une quelconque des revendications précédentes, dans lequel la densité du carton multicouche est inférieure à 800 kg/m3, telle qu'inférieure à 750 kg/m3, telle qu'inférieure à 725 kg/m³.

9. Procédé selon l'une quelconque des revendications précédentes, dans lequel la couche supérieure est formée à partir d'un matériau de remplissage de la couche supérieure comprenant au moins 50 % en poids sec de pâte kraft, tel qu'au moins 80 % en poids sec de pâte kraft.

10. Procédé selon la revendication 9, dans lequel le matériau de la couche supérieure comprend un mélange de pâte de bois dur et de pâte de bois tendre.

11. Procédé selon l'une quelconque des revendications précédentes, dans lequel la couche inférieure est formée à partir d'un matériau de remplissage de la couche inférieure comprenant au moins 50 % en poids sec de pâte kraft, tel qu'au moins 70 % en poids sec de pâte kraft.
